

Nov. 4, 1947.

E. E. NICHOLSON ET AL  
PHOTOGRAPHIC EMULSIONS CONTAINING PSEUDOCYANINE  
DYES AND 9-METHYL THIACARBOCYANINE DYES

2,430,072

Filed Feb. 9, 1945



A=1,1'-DIETHYL-2,2'-QUINO-CYANINE IODIDE.

FIG. 1 P=MIXTURE OF A AND 3,3',9-TRIMETHYL-THIACARBOCYANINE IODIDE.



A=1,1'-DIETHYL-2,2'-QUINO-CYANINE IODIDE.

FIG. 2 T=MIXTURE OF A AND 3,3'-DIETHYL-9,5,5'-TRIMETHYL-THIACARBOCYANINE IODIDE.



A=1,1'-DIETHYL-2,2'-QUINO-CYANINE IODIDE.

FIG. 3 S=MIXTURE OF A AND 3,3'-DIETHYL-9-METHYL-4,5,4',5'-DIBENZ-THIACARBOCYANINE BROMIDE.



B=1,3'-DIETHYL-5'-CHLORO-THIAQUINO (2,2') CYANINE IODIDE.

FIG. 4 P=MIXTURE OF B AND 3,3',9-TRIMETHYL-THIACARBOCYANINE IODIDE.



C=1,3'-DIETHYL-THIAQUINO (2,2') CYANINE IODIDE.

FIG. 5 P=MIXTURE OF C AND 3,3',9-TRIMETHYL-THIACARBOCYANINE IODIDE.



D=1,3'-DIETHYL-5'-METHYL-SELENAQUINO (2,2') CYANINE IODIDE.

Ernest Edward Nicholson INVENTORS  
Ronald Bernard Collins  
BY

Lynn Barratt Morris  
ATTORNEY

## UNITED STATES PATENT OFFICE

2,430,072

PHOTOGRAPHIC EMULSIONS CONTAINING  
PSEUDOCYANINE DYES AND 9-METHYL  
THIACARBOCYANINE DYESErnest Edward Nicholson and Ronald Bernard  
Collins, Ilford, England, assignors to Ilford  
Limited, Ilford, England, a British companyApplication February 9, 1945, Serial No. 577,034  
In Great Britain February 11, 1944

8 Claims. (Cl. 95—7)

1

This invention relates to photographic emulsions and particularly to the manufacture of dye-sensitised photographic silver halide emulsions.

Photographic silver halide emulsions have a certain natural sensitivity to light, but this is restricted to a short range of wavelengths in the ultra-violet and/or blue regions of the spectrum. The effect of incorporating a sensitising dye is to impart to the emulsion sensitivity to light of other wavelengths. It has been known for some time that the effect of incorporating in the emulsion, together with a sensitising dye, a second substance which may or may not itself be a sensitizer, sometimes imparts an additional sensitivity to the emulsion beyond that which can be regarded as the sum effect of the separate substances. Combinations of sensitising dye and another substance which give this latter result are known as supersensitising combinations.

In British Patent No. 498,290 various supersensitising combinations are described, including, among many others, the combination of a pseudocyanine and a carbocyanine containing an alkyl substituent in the central carbon atom of the trimethine chain. These latter compounds are referred to in the said patent as 8-alkyl compounds, but are referred to in the present specification (using the system of numbering which is now preferred and is used in the recent authoritative work "Theory of the Photographic Process" by Mees, published by Macmillan & Co. (1942) as the 9-alkyl compounds.

It is stated in the said patent that the relative quantities of the said two types of compound may vary, for example from 1:5 to 5:1.

It has now been discovered that a very valuable supersensitising effect may be obtained by the combination with an oxa-, thia- or selena-pseudocyanine dye of an extremely small quantity of a 9-alkyl thiacarbocyanine dye, and according to the present invention, therefore, photographic silver halide emulsions are supersensitised by incorporating in the emulsions an oxa-, thia- or selena-pseudocyanine dye in a quantity which alone is sufficient to impart good colour sensitivity to the emulsion, together with a 9-alkyl thia-carbocyanine dye in a quantity which alone would be insufficient to impart any useful colour sensitivity to the emulsion and which is not greater than about  $1/40$  of the weight of the pseudocyanine dye employed.

The optimum quantity of the pseudocyanine dye will vary with the particular emulsion, but will generally be of the order of 50–100 cc. of a 1 in 1000 solution of the dyestuff per 10 litres of

2

emulsion. The quantity of the 9-alkyl thiacarbocyanine dye will accordingly be of the order of  $1\frac{1}{4}$  to  $2\frac{1}{2}$  cc. of a 1 in 1000 solution per 10 litres of emulsion. The invention is of special importance in connection with gelatino silver bromide emulsions, including silver iodobromide emulsions, but may also be employed with emulsions containing silver chloride.

The pseudocyanine dyes employed have the general structure



where R is an alkyl or aralkyl group, A is an acid radicle and X is an oxygen, sulphur or selenium atom. The carbocyclic rings of either or both nuclei may contain substituent groups if desired, e. g. fused benz groups, hydrocarbon groups, alkoxy groups, amino groups or halogen atoms.

The 9-alkyl thiacarbocyanine dyes employed have the general structure



where R<sub>1</sub> is an alkyl or aralkyl group, A is an acid radicle and R<sub>2</sub> is an alkyl group. The carbocyclic rings of the thiazole nuclei may contain substituent groups if desired, for example any of those mentioned in the preceding paragraph. The acid radicles A in the two dyestuffs may be, for example, halogen atoms, alkyl sulphate, alkyl 40 p-toluene sulphonate, or perchlorate radicles, the iodide and bromide radicles being generally preferred. The groups R, R<sub>1</sub> and R<sub>2</sub> are preferably lower alkyl groups, e. g. methyl or ethyl, propyl or butyl, though they may be higher alkyl groups.

The following examples illustrate the invention. In these examples emulsions containing the pseudocyanine dyestuff alone and emulsions containing the pseudocyanine dyestuff together with the 9-alkyl thiacarbocyanine dyestuff were tested for speed to daylight and to "yellow" light. This latter figure was obtained by exposing the test emulsions to white light passing through a filter which cuts off all radiation of wavelengths less than  $520 \text{ m}\mu$  and the increase in the "yellow

speed" shown by the supersensitised emulsions in comparison with the emulsions containing only the pseudocyanine dye affords a measure of the supersensitising effect obtained.

#### Examples

In these examples the following dyestuffs were employed:

##### Pseudocyanine dyestuffs:

- A. 1,1'-diethyl-2,2'-quinocyanine iodide.
- B. 1,3'-diethyl-5'-chloro-thiaquino(2,2')cyanine iodide.
- C. 1,3'-diethyl-thiaquino(2,2')cyanine iodide.
- D. 1,3'-diethyl-5'-methyl-selenaquino(2,2')-cyanine iodide.

##### 9-alkyl thiacyanine dyestuffs:

- P. 3,3'-9-trimethyl-thiacyanine iodide.
- Q. 3,3'-diethyl-9-methyl-thiacyanine iodide.
- R. 3,3'-9-triethyl-5,5'-dichloro-thiacyanine bromide.
- S. 3,3'-diethyl-9-methyl-4,5,4',5'-dibenz-thiacyanine bromide.
- T. 3,3'-diethyl-9,5,5'-trimethyl-thiacyanine iodide.

The combinations of dyes were incorporated in a silver iodobromide emulsion containing about 6.5 gms. of silver halide (calculated as silver) per litre of emulsion, during the manufacture of the emulsion, and the resulting emulsion was coated on glass and the speed values referred to above were determined. The results are set out in the following table:

| Ex-<br>ample<br>No. | Pseudo-<br>cyanine<br>dye | Quantity<br>of Pseudo-<br>cyanine<br>dye in ccs.<br>of 1:1000<br>solution<br>per litre<br>of emulsion | 9-alkyl<br>thiacyanine<br>dye | Quantity<br>of 9-alkyl<br>thiacyanine<br>dye in ccs.<br>of 1:2000<br>solution<br>per litre<br>of emulsion | Day-<br>light<br>speed | Yel-<br>low<br>speed |
|---------------------|---------------------------|-------------------------------------------------------------------------------------------------------|-------------------------------|-----------------------------------------------------------------------------------------------------------|------------------------|----------------------|
| 1a                  | A                         | 6.5                                                                                                   | P                             | 0.25                                                                                                      | 85                     | 9                    |
| 1b                  | A                         | 6.5                                                                                                   |                               |                                                                                                           | 125                    | 51 45                |
| 2a                  | A                         | 6.5                                                                                                   |                               |                                                                                                           | 107                    | 7                    |
| 2b                  | A                         | 6.5                                                                                                   | Q                             | 0.25                                                                                                      | 118                    | 34                   |
| 2c                  | A                         | 6.5                                                                                                   | R                             | 0.25                                                                                                      | 112                    | 17                   |
| 2d                  | A                         | 6.5                                                                                                   | S                             | 0.25                                                                                                      | 170                    | 57                   |
| 2e                  | A                         | 6.5                                                                                                   | T                             | 0.25                                                                                                      | 180                    | 38                   |
| 3a                  | B                         | 10.0                                                                                                  | P                             | 0.25                                                                                                      | 155                    | 14                   |
| 3b                  | B                         | 10.0                                                                                                  |                               |                                                                                                           | 180                    | 37                   |
| 4a                  | C                         | 7.5                                                                                                   |                               |                                                                                                           | 125                    | 17                   |
| 4b                  | C                         | 7.5                                                                                                   | P                             | 0.125                                                                                                     | 125                    | 26                   |
| 5a                  | D                         | 6.5                                                                                                   |                               |                                                                                                           | 185                    | 37                   |
| 5b                  | D                         | 6.5                                                                                                   | P                             | 0.25                                                                                                      | 185                    | 56 55                |

The speed values given in the foregoing table are substantially linearly related, i. e. are in direct proportion.

The supersensitising effects obtained are further illustrated by the accompanying drawings which show spectral sensitivity curves for the emulsions of certain of the foregoing examples. These drawings are as follows:

| Figure No: | Full line   | Dotted line |
|------------|-------------|-------------|
| 1          | Example 1a. | Example 1b. |
| 2          | Example 2a. | Example 2c. |
| 3          | Example 2a. | Example 2d. |
| 4          | Example 3a. | Example 3b. |
| 5          | Example 4a. | Example 4b. |
| 6          | Example 5a. | Example 5b. |

It will be appreciated that the process of this invention presents the clear advantage over the

process described in British Patent No. 498,290 that very much smaller quantities of the supersensitising dye are required, with consequent economic advantage. The results obtained by the present invention are surprising in view of the fact that the quantity of supersensitising dye employed is so small that used alone it does not impart any useful colour sensitivity to the emulsion.

#### What we claim is:

1. A photographic silver halide emulsion containing a pseudocyanine dye selected from the class consisting of oxa-, thia- and selena-pseudocyanine dyes in a quantity which alone is sufficient to impart good colour sensitivity to the emulsion, together with a 9-alkyl thiacyanine-dye in a quantity which alone is insufficient to impart any substantial colour sensitivity to the emulsion and which is not greater than  $\frac{1}{40}$  and not less than  $\frac{1}{120}$  of the weight of the pseudocyanine dye present.

2. A photographic silver halide emulsion containing a pseudocyanine dye selected from the class consisting of oxa-, thia- and selena-pseudocyanine dyes in a quantity of 0.05 to 0.1 gram per 10 litres of emulsion, together with a 9-alkyl thiacyanine-dye in a quantity which alone is insufficient to impart any substantial colour sensitivity to the emulsion and which is not greater than  $\frac{1}{40}$  and not less than  $\frac{1}{120}$  of the weight of the pseudocyanine dye present.

3. A photographic gelatino silver bromide emulsion containing a pseudocyanine dye selected from the class consisting of oxa-, thia- and selena-pseudocyanine dyes in a quantity which alone is sufficient to impart good colour sensitivity to the emulsion, together with a 9-alkyl thiacyanine-dye in a quantity which alone is insufficient to impart any substantial colour sensitivity to the emulsion and which is not greater than  $\frac{1}{40}$  and not less than  $\frac{1}{120}$  of the weight of the pseudocyanine dye present.

4. A photographic gelatino silver bromide emulsion containing a pseudocyanine dye selected from the class consisting of oxa-, thia- and selena-pseudocyanine dyes of 0.05 to 0.1 gram per 10 litres of emulsion, together with a 9-alkyl thiacyanine-dye in a quantity which alone is insufficient to impart any substantial colour sensitivity to the emulsion and which is not greater than  $\frac{1}{40}$  and not less than  $\frac{1}{120}$  of the weight of the pseudocyanine dye present.

5. A photographic gelatino silver bromide emulsion containing a pseudocyanine dye selected from the class consisting of oxa-, thia- and selena-pseudocyanine dyes in a quantity which alone is sufficient to impart good colour sensitivity to the emulsion, together with a thiacyanine substituted in the 9-position by a  $C_nH_{2n-1}$  group where  $n$  is an integer not greater than 4 in a quantity which alone is insufficient to impart any substantial colour sensitivity to the emulsion and which is not greater than  $\frac{1}{40}$  and not less than  $\frac{1}{120}$  of the weight of the pseudocyanine dye present.

6. A photographic gelatino silver bromide emulsion containing a pseudocyanine dye selected from the class consisting of oxa-, thia- and selena-pseudocyanine dyes of 0.05 to 0.1 gram per 10 litres of emulsion, together with a thiacyanine substituted in the 9-position by a  $C_nH_{2n-1}$  group where  $n$  is an integer not greater than 4 in a quantity which alone is insufficient to impart any substantial colour sensitivity to the emulsion and which is not greater than  $\frac{1}{40}$  and not less than  $\frac{1}{120}$  of the weight of the pseudocyanine dye present.

not less than  $\frac{1}{120}$  of the weight of the pseudocyanine dye present.

7. A photographic gelatino silver iodobromide emulsion containing a pseudocyanine dye selected from the class consisting of oxa-, thia- and seleno-pseudocyanine dyes in a quantity which alone is sufficient to impart good colour sensitivity to the emulsion, together with a 9-alkyl thiacarbocyanine dye in a quantity which alone is insufficient to impart any substantial colour sensitivity to the emulsion and which is not greater than  $\frac{1}{40}$  and not less than  $\frac{1}{120}$  of the weight of the pseudocyanine dye present.

8. A photographic gelatino silver iodobromide emulsion containing a pseudocyanine dye selected from a class consisting of oxa-, thia- and seleno-pseudocyanine dyes in a quantity of 0.05 to 0.1 gram per 10 litres of emulsion, together with a 9-alkyl thiacarbocyanine dye in a quantity

which alone is insufficient to impart any substantial colour sensitivity to the emulsion and which is not greater than  $\frac{1}{40}$  and not less than  $\frac{1}{120}$  of the weight of the pseudocyanine dye present.

ERNEST EDWARD NICHOLSON.  
RONALD BERNARD COLLINS.

## REFERENCES CITED

- 10 The following references are of record in the file of this patent:

## UNITED STATES PATENTS

| Number       | Name    | Date          |
|--------------|---------|---------------|
| 15 2,127,340 | Mees    | Aug. 16, 1938 |
| 2,158,882    | Mees    | May 16, 1939  |
| 2,166,938    | Carroll | July 25, 1939 |
| 2,206,076    | Carroll | July 2, 1940  |